# EUROPEAN PATENT SPECIFICATION

(11) **EP 1 375 177 B1**
(45) Date of publication and mention of the grant of the patent: **25.04.2007**
(21) Application number: 03076859.2
(22) Date of filing: 16.06.2003
(51) Int. Cl.: B41M 5/52

(54) **Ink jet recording element and printing method**
Tintenstrahlaufzeichnungselement und Druckverfahren
Elément d'enregistrement par jet d'encre et méthode d'impression

(30) Priority: 26.06.2002 US 180395; 26.06.2002 US 180179
(43) Date of publication of application: 02.01.2004
(73) Proprietor: EASTMAN KODAK COMPANY, Rochester, New York 14650 (US)
(72) Inventor: Sharma, Krishamohan, Eastman Kodak Company, Rochester, New York 14650-2201 (US); Bermel, Alexandra D., Eastman Kodak Company, Rochester, New York 14650-2201 (US); Bringley, Joseph F., Eastman Kodak Company, Rochester, New York 14650-2201 (US); Landry-Coltrain, Christine, Eastman Kodak Company, Rochester, New York 14650-2201 (US)
(74) Representative: Haile, Helen Cynthia

(56) References cited:
- EP-A- 0 391 308
- EP-A- 0 963 947
- PATENT ABSTRACTS OF JAPAN vol. 016, no. 153 (M-1235), 15 April 1992 (1992-04-15) & JP 04 007189 A (KANZAKI PAPER MFG CO LTD), 10 January 1992 (1992-01-10)
- PATENT ABSTRACTS OF JAPAN vol. 017, no. 577 (C-1122), 20 October 1993 (1993-10-20) & JP 05 170425 A (JAPAN SYNTHETIC RUBBER CO LTD), 9 July 1993 (1993-07-09)

## Description

The present invention relates to an ink jet recording element and a printing method using the element containing core/shell particles which improve stability and optical density.

In a typical ink jet recording or printing system, ink droplets are ejected from a nozzle at high speed towards a recording element or medium to produce an image on the medium. The ink droplets, or recording liquid, generally comprise a recording agent, such as a dye or pigment, and a large amount of solvent. The solvent, or carrier liquid, typically is made up of water and an organic material such as a monohydric alcohol, a polyhydric alcohol or mixtures thereof.

An ink jet recording element typically comprises a support having on at least one surface thereof an ink-receiving or image-receiving layer, and includes those intended for reflection viewing, which have an opaque support, and those intended for viewing by transmitted light, which have a transparent support.

An important characteristic of ink jet recording elements is their need to dry quickly after printing. To this end, porous recording elements have been developed which provide nearly instantaneous drying as long as they have sufficient thickness and pore volume to effectively contain the liquid ink. For example, a porous recording element can be manufactured by coating in which a particulate-containing coating is applied to a support and is dried.

When a porous recording element is printed with dye-based inks, the dye molecules penetrate the coating layers. However, there is a problem with such porous recording elements in that the optical densities of images printed thereon are lower than one would like. The lower optical densities are believed to be due to optical scatter which occurs when the dye molecules penetrate too far into the porous layer. Another problem with a porous recording element is that atmospheric gases or other pollutant gases readily penetrate the element and lower the optical density of the printed image causing it to fade.

EP 1 016 543 relates to an ink jet recording element containing aluminum hydroxide in the form of boehmite. However, there is a problem with this element in that it is not stable to light and exposure to atmospheric gases.

EP 0 965 460A2 relates to an ink jet recording element containing aluminum hydrate having a boehmite structure and a non-coupling zirconium compound. However, there is no specific teaching of a metal oxy(hydroxide) complex as described herein.

U.S. Patent 5,372,884 relates to ink jet recording elements containing a cation-modified acicular or fibrous colloidal silica, wherein the cation-modifier is at least one hydrous metal oxide selected from the group consisting of hydrous aluminum oxide, hydrous zirconium oxide and hydrous tin oxide. However, there is no specific teaching of a metal oxy(hydroxide) complex as described herein for a core/shell particle.

JP Publication 04 007189 A (Abstract) discloses an inkjet recording element comprising a support having thereon an image-receiving layer comprising a pigment and a metal(oxy)hydroxide complex exemplified by zirconium salts, but not having a core/shell structure. It does not disclose a core/shell structure.

JP Publication 05 170425 A (Abstract) discloses a composite particle that is suitably used for a catalyst, an adsorbent or an electronic material, including a Y(OH)CO₃ shell on a silica core.

EP-A-0963 947 discloses core-shell composite particles for use in an inkjet recording element in which the core of the core/shell particles is a hydroxy-group-containing material such as magnesium or aluminum hydroxide or porous silica. A shell is formed from an aluminum compound selected from aluminum oxide and aluminum hydroxide.

EP-A-0 391 308 discloses coating a water-insoluble basic alumina salt with a water-soluble basic aluminum as water-resistance improving agent, in order to obtain improved water-resistance and lightfastness.

It is an object of this invention to provide an ink jet recording element that, when printed with dye-based inks, provides superior optical densities, good image quality, image stability, and has an excellent dry time.

Still another object of the invention is to provide a printing method using the above-described element.

These and other objects are achieved in accordance with the invention which comprises an ink jet recording element comprising a support having thereon an image-receiving layer, said ink jet recording element comprising a layer obtainable from a coating composition comprising core/shell colloidal particles in a coating compositon, wherein the core consists of colloidal silica and the shell of said particles consists of 3 to 40 % by weight, based upon the weight of the core particle, of a metal(oxy)hydroxide complex,

Mⁿ⁺(O)ₐ(OH)_{b}(A^{p-})_{c}•xH₂O,

wherein
Mⁿ⁺ is at least one metal ion;
n is 3 or 4;
A^{p-} is present and is an organic or inorganic ion;
p is 1, 2 or 3; and
x is equal to or greater than 0;
with the proviso that when n is 3, then a, b and c each comprise a rational number as follows: 0 ≤ a < 1.5; 0 < b < 3; and 0 < pc < 3, so that the charge of the M³⁺ metal ion is balanced;
and when n is 4, then a, b and c each comprise a rational number as follows: 0 ≤ a < 2; 0 < b < 4; and 0 ≤ pc < 4, so that the charge of the M⁴⁺ metal ion is balanced.

By use of the invention, an ink jet recording element is obtained that, when printed with dye-based inks, provides superior optical densities, good image quality and has an excellent dry time.

Another embodiment of the invention relates to an ink jet printing method comprising the steps of:
A) providing an ink jet printer that is responsive to digital data signals;
B) loading the printer with the ink jet recording element described above;
C) loading the printer with an ink jet ink composition; and
D) printing on the ink jet recording element using the ink jet ink composition in response to the digital data signals.

In a preferred embodiment of the invention, the core/shell particles consist of a core particle having a negative charge upon its surface and having thereon a shell. The size of the core particles may be from 0.01 to 10 µm, preferably from 0.05 to 1.0 µm.

The shell, as described above, comprises 3 to 40 % by weight of the core particle, preferably 10 to 30 % by weight. The shell may have a thickness of 0.005 to 0.500 µm, preferably 0.01 to 0.100 um thick.

In a preferred embodiment of the invention, the core/shell particles described above are located in the image-receiving layer. In another preferred embodiment, M in the above formula is a Group IIIA, IIIB, IVA, IVB metal or a lanthanide group metal of the periodic chart, such as tin, titanium, zirconium, aluminum, silica, yttrium, cerium or lanthanum or mixtures thereof. In another preferred embodiment, n is 4; a, b and c each comprise a rational number as follows: 0 ≤ a < 1; 1 < b < 4; and 1 ≤ pc < 4, so that the charge of the M⁴⁺ metal ion is balanced. In still another preferred embodiment, a is 0, n is 4, and b+pc is 4. In yet still another preferred embodiment, a is 0, n is 3, and b+pc is 3.

In yet still another preferred embodiment of the invention, A^{p-} is an organic anion such as R-COO⁻, R-O⁻, R-SO₃⁻, R-OSO₃⁻ or R-O-PO₃⁻ where R is an alkyl or aryl group. In another preferred embodiment, A^{p-} is an inorganic anionic such as I⁻, Cl⁻, Br⁻, F⁻, ClO₄⁻, NO₃⁻, CO₃²⁻ or SO₄²⁻. The particle size of the complex described above is less than 1 µm, preferably less than.0.1 µm.

Metal (oxy)hydroxide complexes employed herein as the shell material may be prepared by dissolving a metal salt in water and adjusting the concentration, pH, time and temperature to induce the precipitation of metal (oxy)hydroxide tetramers, polymers or particulates upon the core material. The conditions for precipitation vary depending upon the nature and concentrations of the counter ion(s) present and can be determined by one skilled in the art. For example, soluble complexes suitable for preparation of the zirconium (oxy)hydroxide shell materials include, but are not limited to, ZrOCl₂˙8H₂O, and the halide, nitrate, acetate, sulfate, carbonate, propionate, acetylacetonate, citrate and benzoate salts; and hydroxy salts with any of the above anions. It is also possible to prepare the shell materials employed in the invention via the hydrolysis of organically soluble zirconium complexes such as zirconium alkoxides, e.g., zirconium propoxide, zirconium isopropoxide, zirconium ethoxide and related organometallic zirconium compounds.

The hydrolyzed zirconium oxyhydroxides,

Zr(O)ₐ(OH)_{b}(A^{p-})_{c}*xH₂O

may exist as tetrameric zirconia units or as polymeric complexes of tetrameric zirconia, wherein zirconium cations are bridged by hydroxy and/or oxo groups. In general, hydrolyzed zirconia salts are amorphous and may exist predominantly in the α form. However, depending upon the experimental conditions (solvents, pH, additives, aging and heating conditions), the hydrolyzed product may contain significant number of "oxo" bridges.

It is often difficult to ascertain the precise composition of "oxo" and "hydroxy" groups in hydrolyzed metal salts. Therefore, the usage of definitive numbers for these functional groups in metal (oxy)hydroxide compositions was avoided. Any number of oligomeric or polymeric units of metal complexes may be condensed via hydrolysis reactions to form larger particulates ranging in size from 3 nm to 500 nm.

It is further possible to age or heat treat suspensions of the core/shell materials to obtain core/shell particulates ranging in size from 0.500 µm to 5.0 µm. Preferred particles sizes are in the range from 5 nm to 1000 nm. Calcination of amorphous metal (oxy)hydroxide leads to the formation of crystalline polymorphs of metal oxides.

In a preferred embodiment of the invention, the image-receiving layer is porous and also contains a polymeric binder in an amount insufficient to alter the porosity of the porous receiving layer. In another preferred embodiment, the polymeric binder is a hydrophilic polymer such as poly(vinyl alcohol), poly(vinyl pyrrolidone), gelatin, cellulose ethers, poly(oxazolines), poly(vinylacetamides), partially hydrolyzed poly(vinyl acetate/vinyl alcohol), poly(acrylic acid), poly(acrylamide), poly(alkylene oxide), sulfonated or phosphated polyesters and polystyrenes, casein, zein, albumin, chitin, chitosan, dextran, pectin, collagen derivatives, collodian, agar-agar, arrowroot, guar, carrageenan, tragacanth, xanthan, rhamsan and the like. In still another preferred embodiment of the invention, the hydrophilic polymer is poly(vinyl alcohol), hydroxypropyl cellulose, hydroxypropyl methyl cellulose, or a poly(alkylene oxide). In yet still another preferred embodiment, the hydrophilic binder is poly(vinyl alcohol).

In addition to the image-receiving layer, the recording element may also contain a base layer, next to the support, the function of which is to absorb the solvent from the ink. Materials useful for this layer include particles, polymeric binder and/or crosslinker.

The support for the ink jet recording element used in the invention can be any of those usually used for ink jet receivers, such as resin-coated paper, paper, polyesters, or microporous materials such as polyethylene polymer-containing material sold by PPG Industries, Inc., Pittsburgh, Pennsylvania under the trade name of Teslin ®, Tyvek ® synthetic paper (DuPont Corp.), and OPPalyte® films (Mobil Chemical Co.) and other composite films listed in U.S. Patent 5,244,861. Opaque supports include plain paper, coated paper, synthetic paper, photographic paper support, melt-extrusion-coated paper, and laminated paper, such as biaxially oriented support laminates. Biaxially oriented support laminates are described in U.S. Patents 5,853,965; 5,866,282; 5,874,205; 5,888,643; 5,888,681; 5,888,683; and 5,888,714. These biaxially oriented supports include a paper base and a biaxially oriented polyolefin sheet, typically polypropylene, laminated to one or both sides of the paper base. Transparent supports include glass, cellulose derivatives, e.g., a cellulose ester, cellulose triacetate, cellulose diacetate, cellulose acetate propionate, cellulose acetate butyrate; polyesters, such as poly(ethylene terephthalate), poly(ethylene naphthalate), poly(1,4-cyclohexanedimethylene terephthalate), poly(butylene terephthalate), and copolymers thereof; polyimides; polyamides; polycarbonates; polystyrene; polyolefins, such as polyethylene or polypropylene; polysulfones; polyacrylates; polyetherimides; and mixtures thereof. The papers listed above include a broad range of papers, from high end papers, such as photographic paper to low end papers, such as newsprint. In a preferred embodiment, polyethylene-coated paper is employed.

The support used in the invention may have a thickness of from 50 to 500 µm, preferably from 75 to 300 µm. Antioxidants, antistatic agents, plasticizers and other known additives may be incorporated into the support, if desired.

In order to improve the adhesion of the ink-receiving layer to the support, the surface of the support may be subjected to a corona-discharge treatment prior to applying the image-receiving layer.

Coating compositions employed in the invention may be applied by any number of well known techniques, including dip-coating, wound-wire rod coating, doctor blade coating, gravure and reverse-roll coating, slide coating, bead coating, extrusion coating, curtain coating and the like. Known coating and drying methods are described in further detail in Research Disclosure no. 308119, published Dec. 1989, pages 1007 to 1008. Slide coating is preferred, in which the base layers and overcoat may be simultaneously applied. After coating, the layers are generally dried by simple evaporation, which may be accelerated by known techniques such as convection heating.

In order to impart mechanical durability to an ink jet recording element, crosslinkers which act upon the binder discussed above may be added in small quantities. Such an additive improves the cohesive strength of the layer. Crosslinkers such as carbodiimides, polyfunctional aziridines, aldehydes, isocyanates, epoxides, polyvalent metal cations, and the like may all be used.

To improve colorant fade, UV absorbers, radical quenchers or antioxidants may also be added to the image-receiving layer as is well known in the art. Other additives include inorganic or organic particles, pH modifiers, adhesion promoters, rheology modifiers, surfactants, biocides, lubricants, dyes, optical brighteners, matte agents, antistatic agents, etc. In order to obtain adequate coatability, additives known to those familiar with such art such as surfactants, defoamers, alcohol and the like may be used. A common level for coating aids is 0.01 to 0.30 % active coating aid based on the total solution weight. These coating aids can be nonionic, anionic, cationic or amphoteric. Specific elements are described in MCCUTCHEON's Volume 1: Emulsifiers and Detergents, 1995, North American Edition.

The image-receiving layer employed in the invention can contain one or more mordanting species or polymers. The mordant polymer can be a soluble polymer, a charged molecule, or a crosslinked dispersed microparticle. The mordant can be non-ionic, cationic or anionic.

The coating composition can be coated either from water or organic solvents, however water is preferred. The total solids content should be selected to yield a useful coating thickness in the most economical way, and for particulate coating formulations, solids contents from 10-40% are typical.

Ink jet inks used to image the recording elements of the present invention are well-known in the art. The ink compositions used in ink jet printing typically are liquid compositions comprising a solvent or carrier liquid, dyes or pigments, humectants, organic solvents, detergents, thickeners, preservatives, and the like. The solvent or carrier liquid can be solely water or can be water mixed with other water-miscible solvents such as polyhydric alcohols. Inks in which organic materials such as polyhydric alcohols are the predominant carrier or solvent liquid may also be used. Particularly useful are mixed solvents of water and polyhydric alcohols. The dyes used in such compositions are typically water-soluble direct or acid type dyes. Such liquid compositions have been described extensively in the prior art including, for example, U.S. Patents 4,381,946; 4,239,543 and 4,781,758, the disclosures of which are hereby incorporated by reference.

The following examples are provided to illustrate the invention.

### Example 1

### Dye Stability Evaluation Tests

The dye used for testing was a magenta colored ink jet dye having the structure shown below. To assess dye stability on a given substrate, a measured amount of the ink jet dye and solid particulates or aqueous colloidal dispersions of solid particulates (typically about 10%-20.0% by weight solids) were added to a known amount of water such that the concentration of the dye was about 10⁻⁵ M. The solid dispersions containing dyes were carefully stirred and then spin coated onto a glass substrate at a speed of 1000-2000 rev/min. The spin coatings obtained were left in ambient atmosphere with fluorescent room lighting (about 0.5 Klux) kept on at all times during the measurement. The fade time was estimated by noting the time required for complete disappearance of magenta color as observed by the naked eye or by noting the time required for the optical absorption to decay to less than 0.03 of the original value.

### Comparative Coatings C-1 to C-2 (Non-core/shell colloidal particles)

Colloidal dispersions of silica particles were obtained from Nalco Chemical Company. Silica dispersion A had a mean particle size of 112 nm, a pH of 9.6, specific gravity of 1.3 g/ml, and a solids content of 41 %. Silica dispersion B had a mean particle size of 94 nm, a pH of 8.4, specific gravity of 1.3 g/ml, and a solids content of 40 %. The colloidal dispersions were used as received and coated and tested as described above.

### Preparation of Core/Shell Particles

A ZrO(OH)acetate dispersion was obtained from MEI Corporation. The dispersion had 36.5 % solids, an average particle size of less than 10 nm, a pH of 3.8 and a specific gravity of 1.3 g/ml. Core/shell colloidal dispersions were prepared by the simultaneous addition of the silica and zirconium colloidal dispersions into a highly efficient mixing apparatus. The colloidal dispersions were introduced via calibrated peristaltic pumps at known flow rates. The mixing efficiencies and flow rates were varied to obtain stable core/shell colloidal dispersions. The details of the preparation and the characteristics of the dispersions are given below. The mixing efficiency of the apparatus is described by the turnover rate, where the turnover rate = (stir rate(rev/min) x turnover volume (ml/rev)) divided by the aqueous volume. The mixing efficiency was kept constant for each example and was about 25 tumovers/min.

### Inventive Coatings I-1 to I-12 (Core/shell Colloidal Particles)

I-1. Into a 2.0 L container containing 200 ml of distilled water which was stirred with a prop-like stirrer at a rate of 200 rpm was simultaneously added silica colloid A at a rate of 20.00 ml/min for 50 minutes and a zirconium (oxy)hydroxy acetate colloid at a rate of 1.2 ml/min. The weight ratio of the resulting colloid was therefore 95 % silica and 5 % zirconium(oxy)hydroxy acetate. The resulting dispersion had a particle size of 340 nm and settled after standing, indicating that the dispersion was not colloidally stable. The resulting dispersion was then coated and tested as described above and the results shown in Table 1 below.
I-2. This was prepared in an identical manner to that of 1-1, except that the zirconium (oxy)hydroxy acetate colloid was added at a rate of 1.8 ml/min. The weight ratio of the resulting colloid was therefore 92.5 % silica and 7.5 % zirconium(oxy)hydroxy acetate. The resulting dispersion had a particle size of 210 nm and settled after standing, indicating that the dispersion was not colloidally stable. The resulting dispersion was then coated and tested as described above and the results shown in Table 1 below.
I-3. This was prepared in an identical manner to that of I-1, except that the zirconium(oxy)hydroxy acetate colloid was added at a rate of 2.5 ml/min. The weight ratio of the resulting colloid was therefore 90.0 % silica and 10.0 % zirconium(oxy)hydroxy acetate. The resulting dispersion had a particle size of 145 nm and did not settle after standing, indicating that the dispersion was a stable colloid. The resulting dispersion was then coated and tested as described above and the results shown in Table 1 below.
I-4. This was prepared in an identical manner to that of I-1, except that silica colloid B was substituted in place of colloid A, and the zirconium(oxy)hydroxy acetate colloid was added at a rate of 2.5 ml/min. The weight ratio of the resulting colloid was therefore 90.0 % silica and 10.0 % zirconium(oxy)hydroxy acetate. The resulting dispersion had a particle size of 151 nm and did not settle after standing, indicating that the dispersion was a stable colloid. The resulting dispersion was then coated and tested as described above and the results shown in Table 1 below.
I-5. This was prepared in an identical manner to that of 1-1, except that the zirconium(oxy)hydroxy acetate colloid was added at a rate of 4.0 ml/min. The weight ratio of the resulting colloid was therefore 85.0 % silica and 15.0 % zirconium(oxy)hydroxy acetate The resulting dispersion had a particle size of 131 nm and did not settle after standing, indicating that the dispersion was a stable colloid. The resulting dispersion was then coated and tested as described above and the results shown in Table 1 below.
I-6. This was prepared in an identical manner to that of 1-1, except that the zirconium(oxy)hydroxy acetate colloid was added at a rate of 5.6 ml/min. The weight ratio of the resulting colloid was therefore 80.0 % silica and 20.0 % zirconium(oxy)hydroxy acetate. The resulting dispersion had a particle size of 130 nm and did not settle after standing, indicating that the dispersion was a stable colloid. The resulting dispersion was then coated and tested as described above and the results shown in Table 1 below.
I-7 (Reference). This was prepared in an identical manner to that of I-1, except that the zirconium(oxy)hydroxy acetate colloid was added at a rate of 9.3 ml/min. The weight ratio of the resulting colloid was therefore 70.0 % silica and 30.0 % zirconium(oxy)hydroxy acetate. The resulting dispersion had a particle size of 138 nm and did not settle after standing, indicating that the dispersion was a stable colloid. The resulting dispersion was then coated and tested as described above and the results shown in Table 1 below.
I-8 (Reference). This was prepared in an identical manner to that of 1-1, except that silica colloid B was substituted in place of colloid A, and the zirconium(oxy)hydroxy acetate colloid was added at a rate of 9.3 ml/min. The weight ratio of the resulting colloid was therefore 70.0 % silica and 30.0 % zirconium(oxy)hydroxy acetate. The resulting dispersion had a particle size of 93 nm and did not settle after standing, indicating that the dispersion was a stable colloid. The resulting dispersion was then coated and tested as described above and the results shown in Table 1 below.
I-9 (Reference). This was prepared in an identical manner to that of I-1, except that silica colloid B was substituted in place of colloid A, and the zirconium(oxy)hydroxy acetate colloid was added at a rate of 14.5 ml/min. The weight ratio of the resulting colloid was therefore 60.0 % silica and 40.0 % zirconium(oxy)hydroxy acetate. The resulting dispersion had a particle size of 96 nm and did not settle after standing, indicating that the dispersion was a stable colloid. The resulting dispersion was then coated and tested as described above and the results shown in Table 1 below.
I-10. 1.0 g of colloidal silica dispersion B (median particle size 94 nm) was diluted by the addition of 2.0 ml distilled deionized water. 0.23 g of a 14 % (w/w) aqueous dispersion of Yttrium(oxy)hydroxy acetate (median particle size 15 nm) was then added slowly with vigorous stirring. The weight ratio of the resulting colloid was therefore 92.5 % silica and 7.5 % yttrium(oxy)hydroxy acetate. The resulting dispersion had a particle size of 146 nm and did not settle after standing, indicating that the dispersion was a stable colloid. The resulting dispersion was then coated and tested as described above arid the results shown in Table 1 below.
I-11. 1.0 g of colloidal silica dispersion B (median particle size 94 nm) was diluted by the addition of 2.0 ml distilled deionized water. 0.6 g of a 14 % (w/w) aqueous dispersion of Yttrium(oxy)hydroxy acetate (median particle size 15 nm) was then added slowly with vigorous stirring. The weight ratio of the resulting colloid was therefore 82.5 % silica and 17.5 % yttrium(oxy)hydroxy acetate. The resulting dispersion had a particle size of 139 nm and did not settle after standing, indicating that the dispersion was a stable colloid. The resulting dispersion was then coated and tested as described above and the results shown in Table 1 below.
I-12. 1.0 g of colloidal silica dispersion B (median particle size 94 nm) was diluted by the addition of 2.0 ml distilled deionized water. 1.0 g of a 14 % (w/w) aqueous dispersion of Yttrium(oxy)hydroxy acetate (median particle size 15 nm) was then added slowly with vigorous stirring. The weight ratio of the resulting colloid was therefore 74.0 % silica and 26.0 % yttrium(oxy)hydroxy acetate. The resulting dispersion had a particle size of 154 nm and did not settle after standing, indicating that the dispersion was a stable colloid. The resulting dispersion was then coated and tested as described above and the results shown in Table 1 below.

**Table 1**

| Coating | Silica Core Particle | Core/Shell Ratio | Particle Size (nm) | Stable Colloid | Particle Charge | Fade Time |
|---|---|---|---|---|---|---|
| C-1 | A | 100/0 | 112 | Yes | neg. | 18 h |
| C-2 | B | 100/0 | 94 | Yes | neg. | 18 h |
| I-1 | A | 95/5 | 340 | No | neg./pos. | 1 d. |
| I-2 | A | 92.5/7.5 | 210 | No | neg./pos. | 1 d. |
| I-3 | A | 90/10 | 145 | Yes | pos. | 1 d. |
| I-4 | B | 90/10 | 151 | Yes | pos. | 1 d. |
| I-5 | A | 85/15 | 131 | Yes | pos. | 2 d. |
| I-6 | A | 80/20 | 130 | Yes | pos. | 5 d. |
| I-7* | A | 70/30 | 138 | Yes | pos. | > 30 d. |
| I-8* | B | 70/30 | 93 | Yes | pos. | > 30 d. |
| I-9* | B | 60/40 | 96 | Yes | pos. | > 30 d. |
| I-10 | B | 92.5/7.5 | 146 | Yes | NA | 7 d. |
| I-11 | B | 82.5/17.5 | 139 | Yes | NA | > 10 d. |
| I-12 | B | 74/26 | 154 | Yes | NA | > 10 d. |

| | | | | | | |
|---|---|---|---|---|---|---|
| * Reference: not according to present claims | | | | | | |

The above data show that the coatings of the invention containing core/shell particles show improved dye stability (longer time for the dye to lose its optical density) when compared with the non-core/shell comparative coatings.

### Example 2

### Element 1 of the Invention

A coating solution for the base layer was prepared by combining fumed alumina (Cab-O-Sperse® PG003, Cabot Corp.), poly(vinyl alcohol) (Gohsenol® GH-17, Nippon Gohsei Co., Ltd.) and 2,3-dihydroxy-1,4-dioxane (Clariant Corp.) in a ratio of 89:9:2 to give an aqueous coating formulation of 30% solids by weight.

The coating solution for the image-receiving layer was 1-4 described above and poly(vinyl alcohol) (Gohsenol® GH-23A, Nippon Gohsei Co.), and mordant polymeric particles of a copolymer of (vinylbenzyl)trimethylammonium chloride and divinylbenzene (87:13 molar ratio), and surfactant Zonyl® FSN (E. I. du Pont de Nemours and Co.) in a ratio of 73/2/20/5 to give an aqueous coating formulation of 10% solids by weight.

The layers were simultaneously bead-coated at 40°C on polyethylene-coated paper base which had been previously subjected to corona discharge treatment. The image-receiving layer was coated on top of the base layer. The coating was then dried at 60°C by forced air to yield a two-layer recording element in which the thicknesses of the topmost and bottom layers were 2 µm and 40 µm, respectively.

### Element 2 of the Invention

Element 2 of the invention was prepared the same as Element 1 except that the ratio of I-4, poly(vinyl alcohol) (Gohsenol® GH-23A, Nippon Gohsei Co.), mordant polymeric particles of a copolymer of (vinylbenzyl)trimethylammonium chloride and divinylbenzene (87:13 molar ratio), and surfactant Zonyl® FSN (E. I. du Pont de Nemours and Co.) was 67/2/26/5.

### Comparative Elements C-1 to C-4

Comparative Elements C-1 to C-4 were prepared the same as Element 1 except that fumed alumina (Cab-O-Sperse® PG003, Cabot Corp.) was used in place of the core/shell material. The ratios of fumed alumina (Cab-O-Sperse® PG003, Cabot Corp), poly(vinyl alcohol) (Gohsenol® GH-23A, Nippon Gohsei Co.), mordant polymeric particles of a copolymer of (vinylbenzyl)trimethylammonium chloride and divinylbenzene (87:13 molar ratio), and surfactant Zonyl® FSN (E. I. du Pont de Nemours and Co.) for comparative elements 1-4 are listed in Table 2.

### Coating Quality

The dried coatings were visually evaluated for cracking defects.

### Gloss

The dried coatings were measured for 60° specular glossiness using a Gardener® Gloss Meter. A gloss measurement of at least about 60 % is desirable.

### Time

Test images of cyan, magenta, yellow, red, green, blue and black bars, each 1.1 cm by 13.5 cm, were printed using an Epson Stylus® Photo 870 using inks with catalogue numbers C13T007201 and C13T008201. Immediately after ejection from the printer, a piece of bond paper was placed over the printed image and rolled with a smooth, heavy weight. Then the bond paper was separated from the printed image. Ink transferred to the bond paper if the recording element was not dry. The length of the bar imaged on the bond paper was measured. The length of the bar imaged on the bond paper was measured and is proportional to the dry time. Dry times corresponding to a length of about 4 cm or less are acceptable.

**Table 2**

| Element | Ratio* | 60° Gloss (%) | Coating Quality | Proportional Dry Time (cm) |
|---|---|---|---|---|
| C-1 | 67/8/20/5 | 70 | no cracking | 0 |
| 1 | 73/2/20/5 | 74 | no cracking | 0 |
| C-2 | 67/2/26/5 | 75 | no cracking | 0 |
| 2 | 67/2/26/5 | 75 | no cracking | 0 |
| C-3 | 67/8/20/5 | 73 | no cracking | 0 |
| C-4 | 73/2/20/5 | 72 | no cracking | 0 |

| | | | | |
|---|---|---|---|---|
| * Ratio: Particles/polyvinyl alcohol/mordant/Zonyl FSN.® | | | | |

The above results show that all elements had good gloss, coating quality and dry time characteristics.

### Density Testing

Test images of cyan, magenta, yellow, red, green and blue patches at 100% ink laydown were printed on Elements 1 and 2 of the invention and Comparative Elements 1-4 using an Epson Stylus® Photo 870 using inks with catalogue numbers C 13T007201 and C 13T008201. After drying for 24 hours at ambient temperature and humidity, the Status A densities (red, green, blue and visual channels) were measured using an X-Rite® 820 densitometer as follows:

The data in Table 3 show that Examples 1 and 2 employed in the invention had higher densities than the Comparative Elements C-1 to C-2. Comparative elements C-3 and C-4 demonstrate that the density increase cannot be attributed to the level of poly(vinyl alcohol) present in the coating.

## Claims

1. An ink jet recording element comprising a support having thereon an image-receiving layer, said ink jet recording element comprising a layer obtainable from a coating composition comprising core/shell colloidal particles in a coating composition, wherein the core consists of colloidal silica and the shell of said particles consists of 3 to 40 % by weight, based upon the weight of the core particle, of a metal(oxy)hydroxide complex,
Mⁿ⁺(O)ₐ(OH)_{b}(A^{p-})_{c}•xH₂O,
wherein
Mⁿ⁺ is at least one metal ion;
n is 3 or 4;
A^{p-} is present and is an organic or inorganic ion;
p is 1,2 or 3; and
x is equal to or greater than 0;
with the proviso that when n is 3, then a, b and c each comprise a rational number as follows: 0 ≤ a < 1.5; 0 < b < 3; and 0 < pc < 3, so that the charge of the M³⁺ metal ion is balanced;
and when n is 4, then a, b and c each comprise a rational number as follows: 0 ≤ a < 2; 0 < b < 4; and 0 ≤ pc < 4, so that the charge of the M⁴⁺ metal ion is balanced.

2. The recording element of Claim 1 wherein said core/shell particles are present in said image-receiving layer.

3. The recording element of Claim 1 wherein said core/shell particles are present in an overcoat layer.

4. The recording element of Claim 1 wherein M is a Group IIIA, IIIB, IVA, IVB metal or a lanthanide group metal of the periodic chart.

5. The recording element of Claim 1 wherein M is tin, titanium, zirconium, aluminum, silica, yttrium, cerium or lanthanum or mixtures thereof.

6. The recording element of Claim 1 wherein A^{p-} is an organic anion R-COO⁻, R-O⁻, R-SO₃⁻, R-OSO₃⁻ or R-O-PO₃⁻ where R is an alkyl or aryl group.

7. The recording element of Claim 1 wherein A^{p-} is an inorganic anion I⁻, Cl⁻, Br⁻, F, ClO₄⁻, NO₃⁻, CO₃²⁻ or SO₄²⁻.

8. The recording element of Claim 1 wherein said core comprises silica.

9. The recording element of Claim 1 wherein said metal(oxy)hydroxide complex is prepared from an aqueous dispersion having a pH between 3 and 10.

10. An ink jet printing method comprising the steps of:
A) providing an ink jet printer that is responsive to digital data signals;
B) loading said printer with the ink jet recording element of Claim 1;
C) loading said printer with an ink jet ink composition; and
D) printing on said ink jet recording element using said ink jet ink composition in response to said digital data signals.

## Patentansprüche

1. Tintenstrahlaufzeichnungselement mit einem Träger und einer darauf befindlichen Bildempfangsschicht, wobei das Tintenstrahlaufzeichnungselement eine Schicht umfasst, die aus einer Beschichtungszusammensetzung herstellbar ist, die Kern-/Mantel-Kolloidpartikel in einer Beschichtungszusammensetzung umfasst, worin der Kern aus kolloidalem Siliciumdioxid und der Mantel dieser Partikel aus 3 bis 40 Gew.-% eines Metall(oxy)hydroxidkomplexes besteht, bezogen auf das Gewicht der Kernpartikel,
Mⁿ⁺(O)ₐ(OH)_{b}(A^{p-})_{c}•xH₂O,
worin
Mⁿ⁺ für mindestens ein Metallion steht;
n für 3 oder 4 steht,
A^{p-} vorhanden ist und ein organisches oder anorganisches Ion ist;
p gleich 1, 2 oder 3 ist und
x gleich oder größer 0 ist;
mit der Maßgabe, dass für den Fall, dass n gleich 3 ist, a, b und c jeweils eine rationale Zahl wie folgt umfassen: 0 ≤ a < 1,5; 0 < b < 3 und 0 < pc < 3, so dass die Ladung des Metallions M³⁺ ausgeglichen ist;
und für den Fall, dass n gleich 4 ist, a, b und c jeweils eine rationale Zahl wie folgt umfassen: 0 ≤ a < 2; 0 < b < 4; und 0 ≤ pc < 4, so dass die Ladung des Metallions M⁴⁺ ausgeglichen ist.

2. Aufzeichnungselement nach Anspruch 1, worin die Kern-/Mantelpartikel in der Bildempfangsschicht vorhanden sind.

3. Aufzeichnungselement nach Anspruch 1, worin die Kern-/Mantelpartikel in einer Deckschicht vorhanden sind.

4. Aufzeichnungselement nach Anspruch 1, worin M ein Metall der Gruppe IIIA, IIIB, IVA, IVB oder ein Metall der Lanthanidgruppe des Periodensystems ist.

5. Aufzeichnungselement nach Anspruch 1, worin M für Zinn, Titanium, Zirconium, Aluminium, Siliciumdioxid, Yttrium, Zer oder Lanthan oder Mischungen daraus steht.

6. Aufzeichnungselement nach Anspruch 1, worin A^{p-} ein organisches Anion R-COO⁻, R-O⁻, R-SO₃⁻, R-OSO₃⁻ oder R-O-PO₃⁻ ist und R für eine Alkyl- oder Arylgruppe steht.

7. Aufzeichnungselement nach Anspruch 1, worin A^{p-} ein anorganisches Anion I⁻, Cl⁻, Br⁻, F⁻, ClO₄⁻, NO₃⁻, CO₃²⁻ oder SO₄²⁻ ist.

8. Aufzeichnungselement nach Anspruch 1, worin der Kern Siliciumdioxid enthält.

9. Aufzeichnungselement nach Anspruch 1, worin der Metall(oxy)hydroxidkomplex aus einer wässrigen Dispersion mit einem pH-Wert zwischen 3 und 10 hergestellt wird.

10. Tintenstrahldruckverfahren mit folgenden Schritten:
A) Bereitstellen eines Tintenstrahldruckers, der auf digitale Datensignale anspricht;
B) Laden des Druckers mit dem Tintenstrahlaufzeichnungselement nach Anspruch 1;
C) Laden des Druckers mit einer Tintenstrahltintenzusammensetzung und
D) Bedrucken des Tintenstrahlaufzeichnungselements mit der Tintenstrahltintenzusammensetzung in Abhängigkeit von den digitalen Datensignalen.

## Revendications

1. Elément pour l'impression par jet d'encre comprenant un support revêtu d'une couche réceptrice d'image, ledit élément pour l'impression par jet d'encre comprenant une couche pouvant être obtenue à partir d'une composition de couchage comprenant des particules colloïdales de type core/shell (à coeur et à coque) dans une composition de couchage, où le coeur comprend de la silice colloïdale et la coque desdites particules comprend de 3 à 40% en poids, par rapport au poids de la particule du coeur, d'un complexe hydroxyde d'oxyde métallique,
Mⁿ⁺(O)ₐ(OH)_{b}(A^{p-})_{c}•xH₂O,
où
Mⁿ⁺ est au moins un ion métallique ;
n est 3 ou 4 ;
A^{p-} est présent et est un ion organique ou inorganique ;
p est 1, 2 ou 3 ; et
x est égal ou supérieur à 0 ;
à la condition que lorsque n est 3, alors a, b et c représentent chacun un nombre rationnel, tel que : 0 ≤ a < 1,5 ; 0 < b < 3 et 0 ≤ pc < 3, de manière que la charge de l'ion métallique M³⁺ soit équilibrée ;
et lorsque n est 4, alors a, b et c représentent chacun un nombre rationnel, tel que : 0 ≤ a < 2 ; 0 < b < 4 et 0 ≤ pc < 4, de manière que la charge de l'ion métallique M⁴⁺ soit équilibrée.

2. Elément pour l'impression selon la revendication 1, dans lequel lesdites particules de type core/shell sont présentes dans ladite couche réceptrice d'image.

3. Elément pour l'impression selon la revendication 1, dans lequel lesdites particules de type core/shell sont présentes dans une surcouche.

4. Elément pour l'impression selon la revendication 1, dans lequel M est un métal du groupe IIIA, IIIB, IVA, IVB ou un métal du groupe lanthanide de la table périodique.

5. Elément pour l'impression selon la revendication 1, dans lequel M est l'étain, le titane, le zirconium, l'aluminium, le dioxyde de silicium, l'yttrium, le cérium ou le lanthane ou leurs mélanges.

6. Elément pour l'impression selon la revendication 1, dans lequel A^{p-} est un anion organique R-COO⁻, R-O⁻, R-SO₃⁻, R-OSO₃⁻ ou R-O-PO₃⁻, où R est un groupe alkyle ou aryle.

7. Elément pour l'impression selon la revendication 1, dans lequel A^{p-} est un anion inorganique I⁻, Cl⁻, Br⁻, F⁻, ClO₄⁻, NO₃⁻, CO₃²⁻ ou SO₄²⁻.

8. Elément pour l'impression selon la revendication 1, dans lequel ledit coeur comprend du dioxyde de silicium.

9. Elément pour l'impression selon la revendication 1, dans lequel ledit complexe hydroxyde d'oxyde métallique est préparé à partir d'une dispersion aqueuse ayant un pH compris entre 3 et 10.

10. Procédé d'impression par jet d'encre comprenant les étapes suivantes :
A) disposer d'une imprimante à jet d'encre sensible aux signaux de données numériques ;
B) charger dans ladite imprimante l'élément pour l'impression par jet d'encre de la revendication 1 ;
C) charger dans ladite imprimante une composition d'encre pour jet d'encre, et
D) imprimer sur ledit élément pour l'impression par jet d'encre en utilisant ladite composition d'encre pour jet d'encre en réponse auxdits signaux de données numériques.
